

## UNITED STATES PATENT OFFICE

2,001,992

## DYEING ANIMAL FIBERS

Heinrich Wagner, Hans Krzikalla, and Alfred Kirsch, Mannheim, Germany, assignors to General Aniline Works, Inc., New York, N. Y., a corporation of Delaware

No Drawing. Application July 19, 1933, Serial No. 681,216. In Germany July 26, 1932

## 10 Claims. (Cl. 8—5)

The present invention relates to a process of dyeing animal fibers such as skins, hairs, feathers and leather.

We have found that very fast dyeings on animal fibrous materials such as skins, hairs, feathers and leather, are obtained by treating them with solutions of compounds having the general structure



10  
15  
20  
25  
30  
35  
40  
45  
50  
55

wherein R is an alkyl radicle, X<sub>1</sub> and X<sub>2</sub> are hydrogen atoms or members of a benzene nucleus, in the presence of oxidizing agents. Compounds of the kind in question are 1,4-naphthohydroquinone monoalkyl ethers, 1-hydroxy-4-alkoxyanthracenes, and their substitution products, as for example their halogen substitution products. Generally speaking intense blue to green dyeings are obtained on animal fibers by means of the said compounds.

The 1-hydroxy-4-alkoxyanthracenes are obtainable by partial alkylation of 1,4-dihydroxyanthracenes which is attained by treating the said initial materials under mild alkylation conditions, for example by stirring them in the cold for a short time with a solution of hydrochloric acid in the alcohol to be used for etherification. Halogenated derivatives may be obtained by partial alkylation of initial materials containing halogen; for example halogenated 1-hydroxy-4-alkoxyanthracenes can be prepared by partial alkylation of 1,4-dihydroxyanthracenes which are halogenated in the 5-, 6-, 7- or 8- position; the latter compounds may be obtained by reduction of the corresponding quinones.

In order to vary the shades of color other readily oxidizable aromatic compounds containing amino or hydroxyl groups usual for the dyeing of animal fibers may be added to the solutions of the compounds defined above, as for example para-diaminobenzene, para-aminophenol, ortho-aminophenol or alpha-naphthol.

If desired, mordants, as for example iron, copper, chromium or other metal compounds may be employed for mordanting the fibrous materials. In this case some influence on the depth and shade of color of the dyeings may be exerted.

The treatment may be carried out in a neutral or weakly acid medium. It is, however, preferable

to proceed by treating the material to be dyed with a weakly alkaline solution of a hydroxyalkoxy compound as defined above, the oxidizing agent being added to the solution or caused to react before, during or after the introduction of the goods. The treatment with oxidizing agents may also be effected in a separate operation. The desired dyeing may be obtained by hanging the skins or the like impregnated with a 1,4-naphthohydroquinone monalkyl ether or the like in the air, as is usual in the development of vat dyeings. The alkalinity of the caustic soda solution of the 1,4-naphthohydroquinone monalkyl ether or the like may be wholly or partially destroyed by the addition of acids or acid salts or altered by the addition of ammonium salts or ammonia derivatives before or during the dyeing. As a very suitable oxidizing agent may be mentioned in particular hydrogen peroxide, but other oxidizing agents, as for example nitrites, peroxides, such as sodium peroxide and barium peroxide, chromates, persulphates and perborates, may also be employed.

Several of the compounds as defined above may be used together for the dyeing process, for example mixtures of the naphthalene and anthracene derivatives may be employed. The addition of emulsifying agents such as oleyl sulphate, sulphite waste liquor and alkylated naphthalene sulphonic acids, to the dye-bath is very advantageous in many cases.

The dyestuffs formed on the fiber are most probably compounds of the type:



10  
15  
20  
25  
30  
35  
40

wherein R stands for an alkyl radicle and wherein X<sub>1</sub> and X<sub>2</sub> are hydrogen atoms or members of a benzene ring.

The following examples will further illustrate the nature of this invention but the invention is not restricted to these examples.

## Example 1

0.6 kilogram of 1,4-naphthohydroquinone monomethyl ether is dissolved in 6 litres of normal caustic soda solution and diluted with water to form 100 litres of liquor. After adding 10 litres of 3 per cent hydrogen peroxide, the goods to be dyed, skins mordanted by means of potassium

50  
55

- bichromate, are immediately introduced. The dyeing is carried out at room temperature for several hours, very strong reddish blue shades being obtained. Pale to dark blue dyeings are obtained depending on the nature of the mordant. If copper compounds are employed as mordants somewhat less strong greenish blue shades are obtained. If iron mordants are used, a dyeing of dull greenish blue shades somewhat less strong than those obtained with chromium mordants, is produced. It is advantageous to effect the aforesaid process with the addition of 0.3 kilogram of an alkylated naphthalene sulphonate acid or 0.1 kilogram of oleylsulphonate or 0.3 kilogram of a sulphite waste liquor containing 20 per cent of active substance.

*Example 2*

- 0.6 kilogram of 1,4-naphthohydroquinone mono-methyl ether is dissolved in 6 litres of normal caustic soda solution and added to a solution of 5 kilograms of para-diaminobenzene in 100 litres of water. 6 litres of 30 per cent hydrogen peroxide are also added and the goods, as for example skins, are dyed for several hours at room temperature. When employing a skin which has been mordanted with a salt of hexavalent chromium, the hair is dyed a deep black shade and the leather a blue shade. When employing instead of the abovementioned methyl ether the corresponding ethyl or amyl compounds, dyeings of very similar shades are obtained. If leather be used instead of a skin similar dyeings are produced.

*Example 3*

- 0.6 kilogram of 1,4-naphthohydroquinone mono-methyl ether is dissolved in 6 litres of normal caustic soda solution and diluted with water to form 100 litres of liquor. After adding 10 litres of 3 per cent hydrogen peroxide to the dye-bath the goods to be dyed, for example chrome-mordanted skins, are introduced at once. The dyeing is carried out for several hours at room temperature whereby dark-blue shades are obtained on the hairs and the leather of the skins. As soon as the dyeing is finished the skins are removed from the bath and, if desired, rinsed for a short time. Then the skins are introduced while still wet into a dye-bath containing for example 5 kilograms of para-diaminobenzene, dissolved in 100 litres of water and 6 litres of 30 per cent hydrogen peroxide. Deep black shades are obtained on the hairs and blue shades on the leather. Before being introduced into the second dye-bath mentioned the skins may be treated once more with a metal mordant.

*Example 4*

- 0.6 kilogram of 1-hydroxy-4-methoxy- or ethoxy-anthracene is dissolved in about 6 litres of normal caustic soda solution and diluted with water to form 100 litres of liquor. After adding 10 litres of 3 per cent hydrogen peroxide, the goods to be dyed, as for example mordanted skins, are immediately introduced into the liquor. Dyeing is carried on for several hours at room temperature, olive green dyeings being obtained.

Other oxidizing agents, as for example nitrates, peroxides, chromates, persulphates or perborates, may be employed instead of hydrogen peroxide.

Furthermore combination dyeings may be prepared with other oxidizable compounds containing amino or hydroxy groups, as for example para-diaminobenzene, para- or ortho-aminophe-

nol or alpha-naphthol. Displacements in the shade of color may be effected by employing different metallic mordants, as for example iron, copper or chromium compounds.

Instead of 1-hydroxy-alkoxyanthracenes, derivatives thereof, as for example halogenated products, which are capable of being oxidized, may be employed for dyeing.

What we claim is:-

1. The process of dyeing animal fibers, which comprises treating the said fibers with a solution of a compound having the general structure



15

wherein R is an alkyl radicle,  $X_1$  and  $X_2$  are hydrogen atoms or members of a benzene ring, in the presence of an oxidizing agent.

2. The process of dyeing animal fibers, which comprises treating the said fibers with an alkaline solution of a compound having the general structure



30

wherein R is an alkyl radicle,  $X_1$  and  $X_2$  are hydrogen atoms or members of a benzene ring, in the presence of an oxidizing agent.

3. The process of dyeing animal fibers, which comprises treating the said fibers with an alkaline solution of a compound having the general structure



45

wherein R is an alkyl radicle,  $X_1$  and  $X_2$  are hydrogen atoms or members of a benzene ring, in the presence of hydrogen peroxide.

4. Animal fibers dyed with compounds having probably the general structure



55

wherein R is an alkyl radicle and wherein  $X_1$  and  $X_2$  are hydrogen atoms or members of a benzene ring.

5. Animal fibers dyed with compounds corresponding probably to the formula



70

wherein R stands for an alkyl radicle.

75

6. Animal fibers dyed with compounds corresponding probably to the formula

5



10

7. Animal fibers dyed with compounds corresponding probably to the formula

15



20

wherein R stands for an alkyl radical.

8. Animal fibers dyed with compounds corresponding probably to the formula

25



30

9. The process of dyeing animal fibers which comprises treating the said fibers with a solution of a compound having the general structure

5



10

wherein  $X_1$  and  $X_2$  are hydrogen atoms or members of a benzene ring, in the presence of an oxidizing agent.

10. Animal fibers dyed with compounds having probably the general structure

20



wherein  $X_1$  and  $X_2$  are hydrogen atoms or members of a benzene ring.

HEINRICH WAGNER.

HANS KRZIKALLA.

ALFRED KIRSCH.

30

25